

(No Model.)

J. GARNIER.

PROCESS OF EXTRACTING NICKEL FROM ITS OXIDES.

No. 511,886.

Patented Jan. 2, 1894.



Witnesses:  
L. M. Heschelager,  
Henry M. Davis

Inventor  
Jules Garnier,  
By Brisset, Knudz,  
his attorney.

# UNITED STATES PATENT OFFICE.

JULES GARNIER, OF PARIS, FRANCE.

## PROCESS OF EXTRACTING NICKEL FROM ITS OXIDES.

SPECIFICATION forming part of Letters Patent No. 511,886, dated January 2, 1894.

Application filed April 13, 1893. Serial No. 470,147. (No specimens.)

*To all whom it may concern:*

Be it known that I, JULES GARNIER, of the city of Paris, France, have invented an Improved Process for the Extraction of Nickel 5 from its Oxides and Pigs in a Particular Apparatus, of which the following is a full, clear, and exact description.

My invention relates to an improved process for the extraction of nickel from its oxides and pigs in a particular apparatus.

In the metallurgical treatment of nickel according to most of the methods in use, a more or less impure oxide of nickel is obtained, from which it is necessary to extract the metal 15 in as pure a condition as possible, that is to say, practically deprived of carbon, silicon, sulphur, arsenic, phosphorus, &c.

This invention consists of an improved method to obtain this result.

20 The apparatus employed in carrying out the process is illustrated in the accompanying drawings forming part of this specification, in which—

Figures 1 and 2 represent vertical sections 25 thereof taken in planes at right angles to each other.

The apparatus consists of a furnace mounted on trunnions *a b* and having a basic lining *c*, of which the casing *d* is cooled by currents 30 of cold water supplied through the trunnion *a* and pipes *h* to perforated pipes *i* from which it flows down the casing *d* and is collected in gutters *k* at bottom. Hot air is blown in through the trunnion *b* and pipe *e* to the chamber *f* whence it is projected through the tuyeres *y* situated at the side opposite to the pouring off lip. The blowing apparatus is so arranged that it can blow in air at the reduced pressure usual in cupolas, or at the 40 higher pressure necessary in converters. In practice it is preferable to employ two separate blowing machines and to control the blast from the one or the other by means of valves.

Another feature is that for the purpose of 45 cleaning the apparatus the bottom plate *j* is easily removable after first inverting the apparatus and discharging the lumps while still hot, a fresh bottom prepared and heated being then applied and the operation recommenced, and so on.

The object in view is as follows: When the nickel oxide is melted in a cupola furnace, the

nickel is readily reduced but without being carburized, or rather the carbon which combines is almost entirely burned out in front of the tuyeres, or by the oxygen of the oxide, and the result is that the metal adheres to the sides and quickly forms a lump which would not occur were it possible to incorporate carbon and silicon with it. To obviate this objection I first produce by the ordinary processes from a portion of the nickel oxide to be treated, a nickel very rich in carbon and silicon. The apparatus before described having been brought to a white heat, I charge it with alternate layers of bricks of nickel oxide, fuel, and limestone and other fluxes, so as to produce an extra basic and fluid slag containing only from ten to twenty per cent. of silica. The metallic nickel which immediately forms 70 disengages its oxygen which combines with the charges of fuel, but within the sphere of action of the blast from the tuyeres the nickel remains liquid only in consequence of the extremely high temperature, since it has lost its 75 sulphur, a portion of its arsenic and phosphorus (if any) and has not assimilated carbon or silicon in sufficient quantity to give it fluidity. It is at this point that the action of the extra carburized and siliconized nickel 80 before referred to, intervenes to prevent the clogging of the melting chamber, care having been taken to run in this extra carburized nickel before charging it with nickel oxide, so that when the nickel reduced from the oxide reaches the basin of the furnace it there meets with the extra carburized nickel which 85 dissolves it and so prevents the formation of lumps. In running in the carburized nickel, the apparatus is tilted and care is taken to 90 protect the nickel as much as possible from the air by means of wood charcoal thrown upon the fluid metal. Moreover an extra basic slag is first run in, which the carburized nickel must traverse before it reaches the 95 bottom. This slag not only protects the carburized nickel from the oxidizing action of the air but also carries off a considerable proportion of the sulphur it may contain. The carburet of nickel might be charged at the 100 same time as the oxide, but in this case the necessary proportion of carbureted nickel is greater, as the oxide is reduced partly at the expense of the carburet. In any case the

charging is discontinued as soon as the quantity of metal introduced either in the form of oxide or carburet is sufficient to fill the furnace basin to the height of the tuyeres, the charges being melted with a moderate pressure of the blast. Immediately the whole of the metal is collected at the bottom, the apparatus is tilted to discharge the whole of the slag and then returned toward the upright position until the bath reaches the tuyeres when the blast under high pressure is turned on whereby the combustion of the carbon, silicon, arsenic and phosphorus, contained in the metal is effected with formation of fresh slag which is facilitated by adding a certain quantity of lime and fluxes. There still remains in the nickel in intimate admixture therewith a certain proportion of dust from the walls and added lime. The dust of extra basic composition would be prejudicial to the homogeneity of the metal and diminish its strength and to get rid of it the nickel is run on to the silicious hearth of a Siemens furnace in which, after repeated stirrings, this extra basic dust becomes scorified with the silica from the furnace lining. In order to obtain the metal in a practically pure condition there now only remains to add to the bath a deoxidizing agent in as pure a condition as possible, such as ferro-manganese, ferro-aluminium, &c.

It will be understood that the apparatus herein described may be fixed and provided

with two blasts, the scoria and metal being tapped off in the ordinary manner. It will also be evident that this improved method of treatment is applicable to the metallic oxides of cobalt and of iron (residues of the calcination of pyrites, hammer-scale, rich and but slightly silicious ores), to the oxides of chromium and titanium, &c.

I claim—

The process or method of treating oxides of nickel, cobalt, iron, chromium, titanium, &c., which consists in effecting their reduction in a basic apparatus, in contact with extra basic slags and carburizing and silicifying the metal to prevent the formation of a lump by adding a carburet and silicide of said metal; then blowing the metal at high pressure for completing its refinement, and finally running the metal on to the silicious hearth of a Siemens furnace to eliminate the extra basic dust of lime and scoria in mechanical admixture therewith.

The foregoing specification of my improved process for the extraction of nickel from its oxides and pigs in a particular apparatus signed by me this 28th day of March, 1893.

JULES GARNIER.

Witnesses:

DAVID T. S. FULLER,  
ALBERT MOREAUX.